

# UNITED STATES PATENT OFFICE.

MARC EUGENE SANLAVILLE AND RODOLPHE LALIGANT, OF QUINCÉ,  
FRANCE.

## MANUFACTURE OF EXPLOSIVE COMPOUNDS.

SPECIFICATION forming part of Letters Patent No. 281,565, dated July 17, 1883.

Application filed April 8, 1882. (No specimens.) Patented in France April 6, 1881, No. 142,170; in Germany April 11, 1881, No. 19,839; in Belgium April 25, 1881, No. 54,468; in England June 8, 1881, No. 2,488; in Spain August 25, 1881, and in Austria September 17, 1882, No. 18,982.

*To all whom it may concern:*

Be it known that we, MARC EUGENE SANLAVILLE and RODOLPHE LALIGANT, both of Quincé, Department of the Rhône, France, 5 have invented certain new and useful Improvements in the Manufacture of Explosive Compounds, of which improvements the following specification is a full description.

This invention relates to the production of 10 a new class of explosive compounds of such nature that while they possess much greater power than ordinary gunpowder or mining powder, and are equal to dynamite, they can be manufactured and handled with perfect 15 safety.

Explosive compounds, as heretofore employed for mining and military purposes, may be divided into two classes: first, those consisting of a mixture of simple or compound 20 bodies that always have a tendency to combine chemically with each other in being converted more or less completely into a gaseous condition under development of heat and flame, such as the various descriptions of gunpow- 25 der and mining powders; second, those consisting of a chemical combination the elements of which have a constant tendency to become dissociated under development of gas, such as nitro-glycerine. This tendency to combine 30 in the compounds of the first class and to become dissociated in those of the second class renders both classes of explosives very dangerous in their manufacture and use.

The new or third class of explosives, forming 35 the subject of the present invention, is characterized by the fact that the component bodies, whether simple or compound, have, when mixed, no tendency, such as above referred to, either to chemically combine with or become 40 dissociated from each other, it being necessary, in order to bring about the one or the other re- 45 sult, to act upon the compound by means of a re- agent that under the influence of heat shall transform one or more of the component bodies into a condition in which it is or they are free to operate in the manner of either the first or the second class of explosives. By means of this neutral property of the new explosive

and by the method of producing the same, the dangers attendant on the manufacture of explosives of the first class are avoided, the various manipulations and mechanical incorporation of the ingredients of that class, which are a constant source of accidents, being dispensed with. 50

The dangers attendant on the production and use of the second class are also avoided by the fact that the explosive compound is not constituted as such until the moment when the above-mentioned reaction is brought about by 55 the influence of heat. Thus, for instance, if there be introduced into a blast-hole glycerine, together with certain other bodies containing in their composition nitric acid, it will be evident that if, after tamping, the nitric acid be 60 rendered free to combine chemically with the glycerine in the presence of a high degree of heat, nitro-glycerine will be instantaneously produced and explosion will follow. The theoretical formula for such instantaneous for- 65 mation of nitro-glycerine would be as follows, primary mixture:  $3(\text{NaONO}_3 + \text{NaO}_2(\text{SO}_4)_2 \text{HO}) + \text{C}_6\text{H}_{10}\text{O}_6 + (\text{KClO}_3 + 3\text{C})_n$ , giving as first result  $(6\text{NaOSO}_4)_n + \text{n}(\text{KCl}) + 3(\text{CO}_2)_n + 3(\text{NO}_3)_2 \text{HO} + \text{C}_6\text{H}_{10}\text{O}_6$ ; and then as an explosive com- 70 pound  $6(\text{NaOSO}_4)_n + \text{n}(\text{KCl}) + 3(\text{CO}_2)_n + \text{C}_6\text{H}_2(\text{NO}_3\text{HO}) + 3\text{H}_2\text{O}_2$ ; and as the product of explo- 75 sion  $6(\text{NaOSO}_4)_n + \text{n}(\text{KCl}) + 3(\text{CO}_2)_n + 6\text{CO}_2 + 5\text{HO} + 3\text{N}_2 + 3\text{H}_2\text{O}_2$ . In like manner may be shown the production of picrate of potash or ammonia, gun-cotton, and the like. These 80 primary mixtures, as shown by the formulæ, are all preferably harmless, giving compara- 85 tively little or no deleterious or offensive gases by their combustion, as the elements for pro- ducing oxygen can always be present in any sufficient quantity for rendering such combustion complete.

For practically producing the mixture of the bodies containing within them the elements 90 for forming the explosive should be effected, as nearly as practicable, in accordance with the chemical equivalents of those elements. Thus, for obtaining nitro-glycerine as final product at the moment of explosion there should be 95 mixed (A) bisulphate of potash or soda, 36.06

parts, by weight; nitrate of potash or soda, 28.60 parts, by weight; glycerine, 9.20 parts, by weight, together with a second mixture, (B,) chlorate of potash or soda, or other chlorate, 5 fifty parts, by weight; carbonaceous matter, fifty parts, by weight; or, chlorate, fifty-five parts, by weight; carbonaceous matter, forty-five parts, by weight.

It is not necessary that the carbon should be 10 pure. The presence of hydrocarbons, oxygen, and even of nitrogenous matter in small quantity will not sensibly interfere with the reaction.

In the practical manufacture of the new explosive the carbonaceous matter is added to a 15 solution of the salt or salts employed, and when the absorption is complete the mixture is partially dried in a stove. The glycerine is then added to the pasty mass under stirring, and 20 the compound thus obtained is agglomerated and compressed in the form of cartridges, which are inclosed with tarred paper. These should be colored in order to distinguish the description of carbonaceous matter employed. This 25 may be the bran of barley or wheat or other cellulose matter, such as the fibrous tissues of sea-weed.

The ignition of these explosives may be effected by means of a "Bickford" fuse, without 30 requiring any fulminating-priming. They have the peculiar property that the nature of the explosion can be greatly varied, according to the nature of the material upon or purpose

to which the same are to be employed, by varying the quantity of the compound A relatively 35 to the quantity B employed. The greater the quantity of A used the greater will be the proportion of nitro-glycerine generated.

It may be observed that heretofore a mixture has been made of alkaline nitrate, sulphur, 40 and charcoal, (the elements of ordinary gunpowder,) with small quantities of peat and hard coal, metallic sulphates, and animal or vegetable oils or tar, (which elements are said to combine at the time of firing the mixture and 45 form nitro-glycerine.) Such mixture forms no part of the present invention and is not claimed.

What we do claim is—

A composition for use as an explosive, consisting of ingredients such as specified—to wit, 50 carbonaceous matter, alkaline chlorate and nitrate, alkaline bisulphate, and glycerine, or the described equivalent thereof, said materials in admixture being not themselves directly explosive by detonation, but adapted, as 55 the result of their reaction, to produce and immediately to explode nitro-glycerine or similar compound, substantially as described.

In witness whereof we have hereunto signed our names in the presence of two subscribing 60 witnesses.

E. SANLAVILLE.  
R. LALIGANT.

Witnesses:

ROBT. M. HOOPER,  
DE ROUGEMONT.